

# United States Patent Office

2,848,396

Patented Aug. 19, 1958

1

2,848,396

## ELECTROCHEMICAL PREPARATION OF BORON

Nelson F. Murphy and Richard S. Tinsley, Blacksburg, Va., assignors to Callery Chemical Company, Pittsburgh, Pa., a corporation of Pennsylvania

No Drawing. Application February 4, 1955  
Serial No. 486,274

5 Claims. (Cl. 204—60)

This invention relates to the preparation of elemental boron and more particularly to its preparation by the electrolysis of a fused salt mixture containing alkali metal oxides and boron compounds.

Several methods for preparing boron have been developed by various investigators in the past. Moissan first prepared boron in 1892 by the reduction of boric oxide with magnesium. Goss developed a method for preparing boron from boron trichloride and hydrogen. Both these methods are objectionable either because of the low yields obtained or the difficulty of separating the boron from other by-products formed. Cooper in United States Patents 2,572,248 and 2,572,249 produced boron of high purity by the electrolysis of a mixture of potassium salts with or without boric oxide at temperatures of 650°—1000° C. However, he claimed that the use of potassium salts was absolutely essential and that if sodium salts were substituted in whole or in part the process was commercially impractical if not totally inoperative. We have found, however, that when alkali metal oxides are used that either sodium or potassium salts can be used with equal effectiveness.

It is an object of this invention to provide a new and improved method for preparing elemental boron by the electrolysis of a fused salt mixture containing boric oxide, alkali metal fluoborates and alkali metal oxides.

Other objects will become apparent throughout the specification and claims hereinafter related.

This new and improved method will be more fully described in the specification and the novelty thereof will be particularly pointed out and distinctly claimed.

This invention is based upon our discovery that a mixture of boric oxide and an alkali metal fluoborate containing a substantial amount of an alkali metal oxide will produce good yields of elemental boron when electrolyzed at a temperature of 750°—875° C. Since the alkali metal carbonates decompose to the oxide in the presence of  $B_2O_3$  at this temperature, the process is economically attractive.

In carrying out this process, the general procedure was as follows: the salts to be used were weighed, mixed and melted together at about 900° C. in a graphite crucible which was 4" high and had an outside diameter of 4". A calibrated thermocouple was inserted in a hole drilled in the wall of the crucible. The temperature was then lowered to that desired for the experiment. A low-carbon iron rod was used as the cathode which was lowered into the crucible which was used as the anode. The direct current was regulated and electrolysis allowed to proceed for one hour or more with occasional adjustment of heat and current to maintain the desired experimental conditions. Heat was supplied by a gas crucible furnace. At the end of the electrolysis, the current was shut off, the cathode quickly withdrawn and covered with dry sodium chloride to protect the hot product from oxidation. When cool, the cathode was immersed in water until most of the product fell off and the remainder was readily scraped off. The product was digested in hot water for four hours, then

2

refluxed in strong hydrochloric acid, washed again with water, dried and weighted. The weight of the residue was recorded as crude product. The cathode deposits obtained were analyzed for boron as well as carbon and other impurities.

In one series of experiments, a mixture of 2 mols of  $K_2CO_3$ , 2 mols of  $KBF_4$  and 1 mol of  $B_2O_3$  was melted in a graphite crucible at 900°—950° C. until all of the  $CO_2$  was evolved. The temperature was then decreased to 850° C. and a direct current of 15 amperes was passed from the graphite crucible anode to the steel cathode of 4 sq. in. immersed area. After two hours, the steel cathode was removed and cooled under a layer of sodium chloride. The cathode was soaked in water and the deposit removed by scraping it off. The deposit was digested in hydrochloric acid, filtered, washed and dried. The analysis of the product in three separate runs was as follows:

| Run No. | Wt. in grams Crude Product | Percent Carbon | Percent Boron | Percent Oxygen and Other Impurities by Difference |
|---------|----------------------------|----------------|---------------|---------------------------------------------------|
| 1       | 2.68                       | 6.1            | 84.8          | 9.1                                               |
| 2       | 2.84                       | 5.8            | 85.1          | 9.1                                               |
| 3       | 3.45                       | 11.8           | 86.0          | 2.2                                               |

In another series of experiments using a 1:1:1 molar ratio of  $K_2CO_3$  to  $KBF_4$  to  $B_2O_3$  and electrolyzing the mixture at 850°—875° C. using a direct current of 20 amperes for 1.66 hours the following results were obtained:

| Run No. | Wt. in grams Crude Product | Percent Carbon | Percent Boron | Percent Oxygen and Other Impurities by Difference |
|---------|----------------------------|----------------|---------------|---------------------------------------------------|
| 1       | 2.90                       | 10.3           | 79.2          | 11.5                                              |
| 2       | 2.75                       | 11.5           | 88.5          | —                                                 |

In still another series of runs using  $Na_2CO_3$  in place of  $K_2CO_3$  and  $NaBF_4$  in place of  $KBF_4$  in a ratio of 1 mol of  $Na_2CO_3$  to 1 mol of  $NaBF_4$  to 1 mol of  $B_2O_3$  and electrolyzing the mixture at various temperatures with a direct current of 15—20 amperes for various lengths of time the following results were obtained:

| Run No. | Temp., °C. | Time, Hrs. | Wt. in grams Crude Product | Percent Carbon | Percent Boron | Percent Oxygen and Other Impurities by Difference |
|---------|------------|------------|----------------------------|----------------|---------------|---------------------------------------------------|
| 1       | 873        | 1.50       | 2.25                       | 7.3            | 88.7          | 4.0                                               |
| 2       | 770        | 1.00       | 0.20                       | 10.8           | 71.5          | 17.7                                              |

It should be noticed that a low yield and a poor quality product was obtained at a temperature below 800° C. since the bath becomes too viscous for efficient electrolysis. When optimum conditions are used the only appreciable impurity that exists is carbon which results from decrepitation of the graphite crucible and anode. When a separate graphite anode is used instead of using the crucible for an anode the carbon content of the product is markedly reduced.

In another run, a mixture consisting of 1 mol  $K_2CO_3$ , 1 mol  $NaBF_4$  and 1 mol of  $B_2O_3$  was electrolyzed for 1.66 hours at 855° C., using a direct current of 20 amperes. When the resulting product was analyzed, it was found to contain 82.3% boron and 2.3% carbon.

In other experiments, a mixture consisting of a 1:1:1 molar ratio of  $Na_2CO_3$ ,  $KBF_4$  and  $B_2O_3$  was electrolyzed

at 800°-820° C. The products in these runs all contained a high percentage of boron.

Oxygen is the anode product according to the equation  $3M_2O \rightarrow 6M^+ + 1\frac{1}{2}O_2 + 6e^-$ . When a graphite anode is used carbon monoxide is the main anode product from reaction of the anode with the electrochemically produced oxygen according to  $3C + \frac{1}{2}O_2 \rightarrow 3CO$ .

It should be pointed out that the main advantages of this process are: (1) no chlorine is evolved at the anode, (2) potassium salts are not essential, (3) less water is absorbed by the sodium salt mixtures on standing than when potassium salts are used, (4) sodium salt mixtures decrease corrosion of the metal cathode, and (5) the use of sodium salt mixtures reduces erosion of the anode and the crucible.

Having thus described our invention fully and completely as required by the patent statutes, what we desire to claim and secure by United States Patent is:

1. A method of preparing elemental boron which comprises heating a mixture of  $K_2CO_3$ ,  $KBF_4$  and  $B_2O_3$  in a molar ratio of 1:1:1 to 2:2:1 at a temperature in excess of 900° C. until all the  $CO_2$  is evolved, then electrolyzing the resulting fused mixture at a temperature of 850°-875° C. using a graphite anode and a steel cathode and recovering the boron deposited at the cathode.

2. A method of preparing elemental boron which comprises heating a mixture of  $Na_2CO_3$ ,  $NaBF_4$  and  $B_2O_3$  in a molar ratio of 1:1:1 at a temperature in excess of 900° C. until all the  $CO_2$  is evolved, then electrolyzing the resulting fused mixture at a temperature of 750°-875° C. using a graphite anode and a steel cathode and recovering the boron deposited at the cathode.

3. A method of preparing elemental boron which com-

prises heating a mixture of  $K_2CO_3$ ,  $NaBF_4$  and  $B_2O_3$  in a molar ratio of 1:1:1 at a temperature in excess of 900° C. until all the  $CO_2$  is evolved, then electrolyzing the resulting fused mixture at a temperature of about 850° C. using a graphite anode and a steel cathode and recovering the boron deposited at the cathode.

4. A method of preparing elemental boron which comprises heating a mixture of  $Na_2CO_3$ ,  $KBF_4$  and  $B_2O_3$  in a molar ratio of 1:1:1 at a temperature in excess of 900° C. until all the  $CO_2$  is evolved, then electrolyzing the resulting fused mixture at a temperature of 800°-820° C. using a graphite anode and a steel cathode and recovering the boron deposited at the cathode.

5. A method of preparing elemental boron which comprises electrolyzing a fused mixture consisting essentially of boric oxide, alkali metal fluoborate and alkali metal oxide, the molar ratio of alkali metal oxide to alkali metal fluoborate to boric oxide being in the range of 1:1:1 to 2:2:1, at a temperature in excess of 750° C. and recovering the boron deposited at the cathode.

#### References Cited in the file of this patent

##### UNITED STATES PATENTS

25 2,572,249 Cooper ----- Oct. 23, 1951

##### FOREIGN PATENTS

37,559 France ----- Sept. 23, 1930

##### OTHER REFERENCES

Gore: "Chemical Society Journal" (London), vol. 48 (1885 Abstracts), pages 110 and 111.